

April 22, 1930.

R. H. RANGER

1,755,561

PROCESS OF CORRECTING PHOTOGRAPHIC COPIES FOR FACSIMILE TRANSMISSION

Filed Aug. 24, 1925

Fig. 1

EXPOSURE DEVELOPMENT CHART

| MAX.<br>MIN.<br>D<br>D | .60                          | .70                           | .80                           | .90                                      | 1.00                                     | 1.20                                            | 1.40                                              | 1.60                                               |
|------------------------|------------------------------|-------------------------------|-------------------------------|------------------------------------------|------------------------------------------|-------------------------------------------------|---------------------------------------------------|----------------------------------------------------|
| .10                    | 2. SEC. EXP.<br>5. MIN. DEV. | 4. SEC. EXP.<br>4. MIN. DEV.  | 6. SEC. EXP.<br>3½ MIN. DEV.  | 8. SEC. EXP.<br>3. MIN. DEV.             | 32. SEC. EXP.<br>2. MIN. DEV.            | PORTAIT<br>8. SEC. EXP. 1/4 AP.<br>5. MIN. DEV. |                                                   |                                                    |
| .20                    | 1. SEC. EXP.<br>8. MIN. DEV. | 2.5 SEC. EXP.<br>5. MIN. DEV. | 4.5 SEC. EXP.<br>4 MIN. DEV.  | 6.5 SEC. EXP.<br>3.5 MIN. DEV.           | 24. SEC. EXP.<br>25. MIN. DEV.           | COMMERCIAL<br>3. SEC. EXP.<br>3. MIN. DEV.      | PORTAIT<br>32. SEC. EXP. 1/4 AP.<br>2.5 MIN. DEV. |                                                    |
| .30                    |                              | 2. SEC. EXP.<br>10. MIN. DEV. | 3. SEC. EXP.<br>5. MIN. DEV.  | 5. SEC. EXP.<br>4. MIN. DEV.             | 16. SEC. EXP.<br>3. MIN. DEV.            | COMMERCIAL<br>2. SEC. EXP.<br>4. MIN. DEV.      | COMMERCIAL<br>8. SEC. EXP.<br>1. MIN. DEV.        | PORTAIT<br>32. SEC. EXP. 1/4 AP.<br>2.75 MIN. DEV. |
| .40                    |                              |                               | 2. SEC. EXP.<br>20. MIN. DEV. | 4. SEC. EXP.<br>5. MIN. DEV.             | 12. SEC. EXP.<br>3.5 MIN. DEV.           | COMMERCIAL<br>1. SEC. EXP.<br>5. MIN. DEV.      | COMMERCIAL<br>7. SEC. EXP.<br>1. MIN. DEV.        | PORTAIT<br>20. SEC. EXP. 1/4 AP.<br>3. MIN. DEV.   |
| .50                    |                              |                               |                               | PEERLESS<br>5. SEC. EXP.<br>5. MIN. DEV. | 8. SEC. EXP.<br>4. MIN. DEV.             | 32. SEC. EXP.<br>2.25 MIN. DEV.                 | COMMERCIAL<br>6. SEC. EXP.<br>3. MIN. DEV.        | PORTAIT<br>16. SEC. EXP. 1/4 AP.<br>5. MIN. DEV.   |
| .65                    |                              |                               |                               |                                          | PEERLESS<br>6. SEC. EXP.<br>4. MIN. DEV. | 8. SEC. EXP.<br>5. MIN. DEV.                    | 32. SEC. EXP.<br>2.5 MIN. DEV.                    | COMMERCIAL<br>8. SEC. EXP.<br>3. MIN. DEV.         |
| .80                    |                              |                               |                               |                                          |                                          | PEERLESS<br>10. SEC. EXP.<br>3. MIN. DEV.       | 10. SEC. EXP.<br>5. MIN. DEV.                     | 32. SEC. EXP.<br>2.75 MIN. DEV.                    |

CAMERA LENS FULL OPEN WHERE NO APERTURE IS MENTIONED

Fig. 2



INVENTOR  
R. H. RANGER  
BY *W. H. Adams*  
ATTORNEY

## UNITED STATES PATENT OFFICE

RICHARD HOWLAND RANGER, OF BROOKLYN, NEW YORK, ASSIGNOR TO RADIO CORPORATION OF AMERICA, A CORPORATION OF DELAWARE

## PROCESS OF CORRECTING PHOTOGRAPHIC COPIES FOR FACSIMILE TRANSMISSION

Application filed August 24, 1925. Serial No. 51,930.

This invention relates to certain new and useful improvements in the transmission of facsimile messages, and more especially to a process for improving the detail of transmitted facsimiles and to a process for producing a film of the facsimile to be transmitted which is adapted to give the best results, particularly when the transmission is carried on according to the method disclosed 10 and claimed in my copending application, Serial No. 726,235, filed July 16, 1924 for "Duplex photo modulator".

In the said application I have shown a method and apparatus whereby variations of 15 light intensity corresponding to successive areas of the facsimile to be transmitted are translated into impulses varying in length or spacing according to light intensity.

It has been found that in general films 20 which are supplied to be transmitted vary greatly, not only in light intensity, but in the range of light intensity which may be covered by the high lights and shadows of particular pictures. For example, to ex- 25 press this in a quantitative way, if we designate the intensity of light falling on the film by  $L_o$  and the intensity of light transmitted therethrough by  $L_t$ , then we may express the 30 opacity of the film or the ratio of light which it transmits to that which falls upon it as  $\frac{L_t}{L_o}$ .

It will be seen that if the film is entirely 35 transparent or perfectly clear, the light transmitted through it will be substantially equal to that falling upon it and the ratio in this case will have a value of unity. If, on the other hand, the film is very dark, for 40 instance almost black, the light transmitted through the film may be only perhaps 1/100 of the light falling upon it and the ratio in this case would be 100.

For certain purposes it is desirable to consider, not this ratio itself, but the logarithm 45 of this ratio to the base 10, which is termed "density".

From the foregoing, it will be understood 50 that a film of zero density is a film which is perfectly clear and that a film of 2.0 density is practically opaque. It will also be seen

that intermediate values of this density will lie along a logarithmic scale from opaque to clear.

In carrying out the transmission of facsimiles, and more particularly pictures, in accordance with my invention above referred to, I have found that all films are not transmitted equally well, but that the best results are obtained by the use of what may be termed a "thin" film; that is to say, one in which the opacity is relatively low throughout the picture and in which the density varies between 0.1 and 0.8 approximately, or in other words, a standard picture or film. As a rule, photographic films do not fall within this range, but are normally much more dense both in high lights and shadows and likewise the average range of density, or the contrast, is greater.

If such films were transmitted, a certain amount of detail would therefore be lost. To obviate this, in accordance with my invention I produce from the film to be transmitted a copy falling within the range desired. It might of course be possible to produce a copy having the desired range by a method of "cut and try." This however would be uneconomical and inefficient and I have therefore devised a method and apparatus for determining first of all the density range of any film desired to be transmitted, and secondly for determining under what conditions the copying of the film should be carried out to produce a film having the density range found by experience to be best.

In view of the foregoing, it will now be understood that it is an object of this invention to produce a method and apparatus for utilizing a facsimile transmission system to the best advantage.

It is a further object of this invention to produce a method and apparatus whereby any film may be copied to produce a film lying within a predetermined density range.

It is a further object of this invention to produce a method and apparatus for eliminating guess work and wastage in attempting to produce a film having a desired density range.

Still further objects of my invention will be apparent from the specification.

My invention will best be understood by reference to the following description taken in connection with the accompanying drawing, in which:—

Fig. 1 is a reference chart used in carrying out my invention, and

Fig. 2 is a curve showing the range of contrast of various photographic materials.

In accordance with my invention, I first take the film which it is desired to transmit and measure its density range on what may be termed a "densitometer." The precise construction and arrangement of a densitometer forms no part of this invention. A suitable densitometer may consist of a standard light focusing its beam on a calibrated measuring scale having a variety of densities or on the film to be measured. This light beam is then thrown by suitable optical means on a photo cell and the current variations produced by changes in light intensity are applied to the grid of a three-electrode vacuum tube in such a manner as to change the grid voltage of this tube and consequently the plate current from which the density may be determined by comparison with the standard densities.

Having determined as distinguished from merely estimating, the density range of the film desired to be transmitted, we may proceed to copy it in such a manner as to give the desired density range in the copy, as will be more particularly described.

I have found that the density range in any film copy is dependent upon a number of factors, for example, time of exposure, time of development, type of film, etc. The slower types of film result in a copy having a much greater range of density than a fast film for the normal exposure for each type. Also, it will be found that short exposures of varying light intensity will give a range of density values different from long exposures of the same varying light values. In general it will be found that the longer the exposure from a light of a given intensity, the greater will be the density of all parts of the picture and for a very extreme exposure the film could be converted into a uniformly opaque layer.

The different in intensity between the portion of the film receiving the strongest illumination and the portion receiving the weakest illumination depends upon the length of time of development. It is found that with a given exposure a short time of development will produce a certain density in the portions receiving the least light and a greater density in the portions receiving the most light. An increase in development time will produce a greater density in the portions receiving the least light and a proportionately much greater density in the portions receiving the most light. It is, therefore, possible

to control the range of contrast between the maximum and minimum densities of the film by a variation in development time. It is also possible to control the density of any given part of the film or the average density by varying the exposure.

From this it will be seen that by varying the length of time of exposure and the length of time of development the density range and the maximum and minimum densities can be brought to a desired value.

For instance, referring to Fig. 1, in which abscissae designate maximum density and ordinate designate minimum density, it will be seen that to obtain a film of the desired range from a film having a maximum density of .60 and a minimum density of .10, it is necessary to give a two seconds exposure and to develop for five minutes. On the other hand, to obtain a film of the desired range from a film having a maximum density of 1.0, and a minimum density of .1, it is necessary to give an exposure of 32 seconds, greatly in excess of that required for the first example. To prevent shifting the whole film down the scale towards black, development time is only two minutes, as will be seen.

To give another example, suppose it is desired to produce a film for transmission from a film having a maximum density of .70 and a minimum density of .10, by reference to the chart it will be seen that a four seconds exposure is required and four minutes development. On the other hand, if the film to be copied has a maximum density of .70 and a minimum density of .30 only two seconds exposure is required, but 10 minutes development is necessary.

The examples just given and the blocks on the chart of Fig. 1 in which no film is mentioned are given for Eastman Process Films and Eastman Process Developer at a temperature of 70° Fahrenheit with camera lens full open where no aperture is mentioned.

Certain pictures when submitted, however, are found to have such a contrast or range of density that it is not possible to produce a suitable film for transmission by the process just mentioned. Such films can, however, be reproduced to give a satisfactory film for transmission by choosing another type of sensitized film. For instance for a film having a maximum density of 1.20 and a minimum of .20, an Eastman commercial film may be used giving it three seconds' exposure and three minutes' development.

The factors governing the choice of film to be made to secure a suitable reproduction are indicated by the curves of Fig. 2 which show the difference in density obtained in the completed copy from a given original when different types of film are used. From these curves it will be evident that a certain film marked "A" would give only a very small range of density when the original from

which the copy is made has a wide range of transparency, while another film which may be indicated as film "R" will give a very wide range of density when used to make a copy of the same original.

It is possible of course to make use of special developers to accomplish other changes, but I have found the most practicable process to be the use of a fast developer at a fixed temperature and to use generally only one type of film to cover most of the ranges and then to use extra contrast films for the lowest contrast originals, such as is shown for instance by the use of Peerless film for an original having a maximum density of 1.0 and a minimum density of .55. Also, it may be stated that special ranges may be taken care of by varying the aperture of the lens, in making the copy.

While I have disclosed and claimed the method of preparing pictures for electrical transmission, it is to be distinctly understood that the subject matter transmitted may be in addition to pictures, checks, finger prints, financial statements, newspaper articles, motion picture films and the like, and, in fact, all other matter which is capable of being read or viewed by the eye, and, therefore, I believe that the term "picture", as used throughout the specification and claims, should be broadly construed and considered as broadly relating to all of the various steps to be hereinafter defined and set forth.

While I have shown but a single embodiment of the method of my invention, it is capable of modifications therefrom and it is desired therefore that only such limitations shall be imposed thereon as are required by the prior art or indicated by the appended claims.

I claim:

1. The method of preparing a picture for electrical transmission of a facsimile thereof, which comprises, optically determining the average density range of said picture, comparing said picture with a predetermined schedule of density range obtained from a standard picture having an optimum density range for electrical facsimile transmission, reproducing said first picture to secure a copy thereof having substantially the same density range as said second picture, and electrically transmitting a facsimile of said copy.

2. The method of preparing a picture for electrical transmission of a facsimile thereof, which comprises, optically determining the density range of said picture, comparing said picture with a predetermined schedule of density range obtained from a standard picture having optimum density range for electrical facsimile transmission, reproducing said first picture to secure a copy thereof having substantially the same density range as said second named picture, and electrically transmitting a facsimile of said copy.

3. The method of preparing a picture for electrical transmission of a facsimile thereof, which comprises, optically determining the average density range of said picture, comparing said picture with a predetermined schedule of density range obtained from a standard picture having an optimum density range for electrical facsimile transmission, determining the ratio of density range between said picture and said standard from said comparison, reproducing said first named picture to secure a copy thereof having a density range varying in accordance with the said ratio, and electrically transmitting a facsimile of said copy.

4. The method of preparing a picture for electrical transmission and facsimile thereof, which comprises, optically measuring the optimum range of density in a standard picture for electrical facsimile transmission, optically measuring the range of density in a second picture to be transmitted, determining the ratio of the respective ranges of light intensities in said pictures, producing a copy of said second picture under conditions adjusted in accordance with the ratio of light intensities of the two said pictures, and electrically transmitting a facsimile of said produced copy.

5. The method of preparing a picture for electrical transmission of a facsimile thereof which includes optically determining the average density range of said picture, comparing the density range of said picture with a predetermined schedule of density range obtained from a standard picture having an optimum density range for electrical facsimile transmission, reproducing said picture to secure a copy thereof having an optimum density range varying between 0.1 and 0.8 and having a relatively low opacity, and electrically transmitting a facsimile from such copy.

RICHARD H. RANGER.

110

115

120

125

130